# EUROPEAN PATENT SPECIFICATION

(11) **EP 0 694 094 B1**
(45) Date of publication and mention of the grant of the patent: **03.09.1997**
(21) Application number: 94911975.4
(22) Date of filing: 15.04.1994
(51) Int. Cl.: D06M 11/82, E04B 1/94

(54) **FIBROUS PRODUCTS AND A PROCESS FOR PREPARING FLAME RETARDANT FIBROUS PRODUCTS**
FASERIGE PRODUKTE UND VERFAHREN ZUR HERSTELLUNG VON FLAMMHEMMENDEN FASERIGEN PRODUKTEN
PRODUITS FIBREUX ET PROCEDE DE PREPARATION DE PRODUITS FIBREUX NON INFLAMMABLES

(30) Priority: 15.04.1993 FI 931721
(43) Date of publication of application: 31.01.1996
(73) Proprietor: EKOVILLA OY, SF-45720 Kuusankoski (FI)
(72) Inventor: LOUKO, Reijo, FIN-45700 Kuusankoski (FI); AHONEN, Heikki, FIN-37630 Valkeakoski (FI)
(74) Representative: Cummings, Sean Patrick
(86) International application number: FI9400142
(87) International publication number: WO9424359

(56) References cited:
- EP-A- 0 500 999
- WO-A-93/04239
- FI-B- 73 704
- GB-A- 1 100 982
- GB-A- 1 321 514
- GB-A- 2 093 875
- US-A- 4 374 171

## Description

The present invention relates to a method according to the preamble of claim 1 suited for manufacturing fibrous products made from organic fibers.

According to said method, the fibrous raw material is defibered to a desired degree of defibering and a fire-retardant agent is admixed with it to the end of manufacturing a product of essential flame-retardancy.

The invention also concerns an essentially fire-retardant organic fiber-based material according to claim 8.

Such a material is comprised of organic fibers milled to a desired degree of defibering and admixed with a fire-retardant agent.

The material according to the invention is suited for use particularly as a thermal insulation and also as an aggregate in, e.g., road pavement materials and similar materials applied in hot form.

Recycling and reuse of waste materials have gained a wide importance in today's industrialized world. To utilize recycled paper, methods have been developed permitting the reuse of such fibers in the manufacture of, e.g., thermal insulation materials. These insulation materials include products called, among other names, as cellulosic blow wool or Ecowool, are widely marketed and a plurality of patents related thereto are known. In fact, since 1977 in the USA alone, the patents granted cover 50 types of thermal insulation materials made from wood fiber, the composition of fire retardant agents used with such materials and manufacturing methods thereof, as well as binding agent compositions used for spray-bonding of the said fibers. Some of the patents also teach the sterilization of said cellulosic wool insulation material to the end of improving its resistance against decay in the insulation cavity.

The thermal insulation capability of materials used for thermal insulation of buildings is based on the fact that the insulation material prevents air circulation in the insulation cavity. An ideal insulation material would be characterized by also to a certaing extent being capable of preventing the random movement of molecules in the air. The latter category includes insulation materials termed aerogels in which the pore size is in the order of a few nanometers. The insulation performance can also be improved by filling the voids in the insulation material with a gas of low thermal conductivity or such materials that provide a high reflectance to IR radiation and are inferior heat conductors. Obviously, the most effective thermal insulation is a vacuum complemented with a plurality of high-reflectance surfaces spaced from each other. However, such exotic materials cannot be economically used in these days for the thermal insulation of a conventional building or similar structure.

The thermal conductivity of air is 0.0253 W/m°C, which value can be closely attained by expanded polystyrene having a plurality of reflecting surfaces and a small pore size. The best material available from natural sources which is cork that has a thermal conductivity in the order of 0.045 W/m°C at a density of 140 kg/m³.

The thermal conductivities of typical cellulosic insulation wool, or Ecowool, are approx. 0.034 - 0.036 W/m°C at best. Correspondingly, the thermal conductivity of, e.g., mineral wool is in the order of 0.040 W/m°C, sometimes 0.038 W/m°C. Respectively, the advantageous densities are 30 - 36 kg/m³ for cellulosic wool and 30 - 80 kg/m³ for mineral wool. The difference is related to the different values of thermal conductivity. As for many other materials, the best insulation results are obtained using a density of 40 - 60 kg/m³ for the mineral wool.

The benefits of thermal insulation products made from organic fibers in regard to, e.g., mineral wool insulation materials are their high thermal insulation capability and advantageous production costs. Owing to the possibility of using recycled paper as the raw material, the competitive edge of these products will be further improved in the future.

Typically, cellulosic insulation wool is made by shredding paper and milling the shreds by means of, e.g., a hammer mill and admixing the milled fibers with a fire-retardant agent to render the insulation wool noncombustible and nonsmouldering. Simultaneously, a great number of the fire-retardant agents used therein also act as fungicidal and antimicrobial agents that inhibit the growth of such microorganisms. Typical of such agents are boron compounds, salts of phosphoric acid, antimony compounds, urea etc., that is the same agents that are conventionally used in all other applications of fire resistance improvement.

As an example of the prior art, reference is made to US patent publication 4,804,695 comprising milling fibrous raw material, which can be either wood or (recycled) paper, together with pulverized boric acid (adding boric acid by 14 % of the weight of the fibers) using a hammer mill for the milling step.

Concurrent processing techniques of cellulosic wool have some drawbacks. Namely, the hammer mill crushes the fibers but does not defiber them in the same manner as purpose-designed refiners. Such crushing of the fiber converts it to a form which is disadvantageous in terms of the thermal insulation function.

Further, it would be advantageous in terms of production to blend all required chemicals such as the fire-retardant agents and preservation chemicals already prior to the milling step in order to ensure their homogeneous mixing with the base material. This, however, is not possible when using defibering refiners. The reason is as follows:

Typical fire-retardant agents such as borax or boric acid or soda or mixtures thereof are used in hydrated form to exploit their fire-retardant capability. In fact, borax and other similar chemicals are preferably used as fire-retardant agents particularly in their hydrated forms as then the water of hydration is released at the lowest possible temperature thus absorbing heat and capturing oxygen from the surroundings of the fiber in a fire situation. Alternatively, if admixed with the base material in anhydrated form, anhydrated borax or other similar chemical capable of absorbing water of hydration can later absorb the water of hydration assuming that the required water of hydration is available from, e.g., the humidity of the surrounding air.

The ten waters of hydration bound by hydrated borax are first released at 60.8 °C temperature when the borax is converted into pentahydrate and/or tetrahydrate, and later at 95 °C to dihydrate. When milling recycled paper, for instance, the dry milling step is conventionally carried out using a specific input energy of approx. 100 kWh per ton of raw material. Already at such a relatively low level of specific input energy, the internal temperature of the fibrous material and the temperature of entrained air and additives are elevated so much as to cause the "melting" of hydrated chemicals in their contained water of hydration, whereby plugging of all grooves in the refiner bars results.

In addition to the actual production costs of insulation materials, the *in situ* installation of the insulation material forms a significant factor in the thermal insulation costs of buildings.

The lowest-cost installation method of thermal insulation is blowing by means of an air flow to the insulation cavities. Cellulosic wool and other blowable insulation materials are conventionally best suited for use in applications involving insulation of such horizontal surfaces on which a certain degree of long-term self-compressive settling is not crucial. Due to this reason, the major market for these insulation materials has principally been in the insulation of attic floors of buildings, and also to some extent, of ground floors. By contrast, these insulation materials which tend to settle under self-compression have rarely been used as such in the insulation of wall cavities.

When blowing a loose-fill material such as cellulosic wool or mineral wool into a cavity to be insulated in the wall of a building, the above-described reasons have invariably necessitated the coapplication of a binder suited to bind the fibers together so as to prevent the settling of the installed insulation.

However, such addition of binding agents brings about several drawbacks including:
- unavoidable introduction of moisture into the space to be insulated,
- higher consumption of fire-retardant agent(s) due to added binding agents,
- problems incurred by volatile chemicals contained in the binding agents or from the acting of such agents as a favoured nutrient for microbes and fungal hyphae.

It is an object of the present invention to overcome the disadvantages of the prior-art technology and to achieve an entirely novel method of manufacturing such organic fiber-based products which are suited for use as, e.g., blowable thermal insulation materials and aggregates in various compositions applied in hot form.

The invention proposes a method as claimed in claim 1.

According to the present invention, a fibrillated fibrous product is produced by milling a suitable cellulosic or lignocellulosic raw material in the manner described below. The cheapest product is achieved by defibering recycled paper, while the method is also suited for making products directly from wood or virgin pulp/paper.

The recycled paper can be either groundwood-containing, that is, newsprint essentially consisting of paper made from mechanical pulp, or groundwood-free paper which is printing paper essentially made from chemical pulp, or alternatively, paper containing both of these pulp types such as LWC paper principally made from mechanical pulp with chemical pulp admixed as a strength-imparting component. Furthermore, the recycled paper may contain fillers and pigments, or alternatively, be essentially free from these.

All the above-listed raw material grades are termed as "fibrous raw material" in the context of the present invention. The term "paper" is defined to include all grades of paper, paperboard, cardboard and board with a basis weight in the range of 50 - 500 g/m² typical.

In a preferred embodiment of the invention, in which recycled paper is processed into a thermal insulation material, a particularly suitable fibrous raw material is formed by paper at least essentially made from lignocellulosic (wood-containing) pulp. An example of such raw material is recycled newsprint. According to a second preferred embodiment of the invention, in which an aggregate for, e.g., asphalt is produced, a particularly suitable fibrous raw material is coated paper containing besides pulp, also mineral fillers such as clay and/or talc. This kind of paper includes, e.g., archive-proof copying papers, magazine papers, art printing papers, etc. The end product contains after milling approx. 1 - 50 % clay, talc or similar mineral-based filler used in printing papers.

The fibrous raw material is ground to desired degree of defibering. In this context, "desired degree of defibering" refers to fibrillation of the fibrous raw material in smaller particles. The target size of the particles varies according to the application.
Accordingly, in the first preferred embodiment of the invention mentioned above, the raw material is ground to a particle size of approx. 0.1 - 50 mm, advantageously approx. 1 - 10 mm. In the second preferred embodiment of the invention, the raw material is ground to a much smaller particle size of typically approx. 0.01 - 10 mm, advantageously approx. 0.1 - 5 mm.

For the end result of the milling step it is essential that an attrition action is attained which leads to the defibering of the raw material fibers, whereby a product resembling fluff (or ripped pulp) is obtained.
Accordingly, suitable mills are disk or conical refiners and similar refiner types having rotary refining plates or knives. Particularly advantageously the refiners are equipped with grooved or tipped bars. As will be described below, a particularly advantageous embodiment employs for the defibering of recycled paper such grooved bars in which the grooves are approx. 5 mm deep and the ridges are 3 - 5 mm high. Milling with grooved bars can provide a product of finer degree of defibering than, e.g., tipped bars. In the refiner used herein, the typical bar clearance is in the order of 0.1 - 0.5 mm for defibering recycled paper.

In conjunction with the present invention it has been found that disk and conical refiners can also be employed for admixing the raw material to be milled with the fire-retardant agents such as borax, boric acid, soda, urea, alkali metal salts of phosphoric acid, etc., provided that these agents are introduced in anhydrated or almost anhydrated form. Particularly advantageous fire retardants are borax, soda or a mixture thereof. Agents advantageously suited for use as fire retardants are salts occurring in forms including at least five waters of hydration, advantageously ten waters of hydration, as well as also in anhydrated forms or forms with a lesser amount of waters of hydration. An essential portion of said waters of hydration of said salts is released at a temperature above 30 - 120 °C.

"Fire retardancy" in this context refers to reduction of the inflammability of a material, that is, conversion of the material to a form which is at least essentially noncombustible and nonsmouldering.

The fire-retardant action of agents mixed in dry form is not as effective as that of compounds containing water of hydration. Consequently, according to the present invention, it has been found advantageous to introduce the fire-retardant agent in two portions: in its anhydrous form and hydrous form. Accordingly, a portion which is 1/4 - 1/2 of the fire-retardant material is introduced in anhydrous form to the fibrous base material prior to defibering, and the other portion which is 1/2 - 3/4 of the fire-retardant material is introduced in hydrous form to the fibrous base material after defibering.

If the entire amount of fire-retardant agents is admixed in dry form with the base material fibers in conjunction with the milling step, a greater amount of the fire-retardant agent(s) is required to ensure the initial fire retardancy of the thermal insulation material. Moreover, it must be noted that not all of the fire-retardant agent can be admixed in anhydrous form with the fibrous material, because such a procedure makes it difficult to prevent plugging of the grooved bars. In fact, it has been found that, e.g., anhydrous borax can be maximally admixed with the fibers prior to the milling step by only approx. 8 % of the weight of the fibrous raw material and still keep the bars clean and unplugged. Of course, several different types of refiner bars are used, but the above-given guideline is valid for bars having an approx. 5 mm deep groove and a 3 - 5 mm high ridge that have been found to render an optimal result in the dry-defibering of recycled paper. The advantageous choice of this bar type is evidenced in that such bars make it possible to produce thermal insulation material having a density of 30 kg/m³, while thermal insulation material produced using tipped bars or a hammer mill gives a density of 36 kg/m³ for the insulation material.

As a general rule, the upper limit for the admixed amount of anhydrous borax or similar fire-retardant agent is approx. 10 - 15 % of the weight of the fibers.

During the milling step, the raw material is advantageously admixed with another material, particularly such that also itself becomes milled. Hence, the fire-retardant agents are complemented or augmented preferably using other anhydrous or hydrous salts to the end of fixing other materials to the raw material fibers.

The method according to the invention achieves the following benefits and others:
- A portion of the fire-retardant agent can be better dispersed between the fibers.
- A disk or conical refiner equipped with grooved or tipped bars can be used.
- The dry fibrous material will later become moist, that is, accumulate water of hydration, whereby the insulation material swells and undergoes mutual binding of the fibers thus providing a nonsettling insulation structure.
- The dry, well-dispersed material, which initially is anhydrous but later becomes hydrous through absorbing water of hydration, forms a good substrate also for other agents that can be easily bound to the fibers.

In the present context, the last item above particularly refers to activated carbon.

Namely, elimination of radon hazard can be advantageously achieved according to the present invention. As the thermal insulation of buildings is improved resulting in greater tightness of the building, a growing problem arises from the isolation of radon gas entering the building. When the ground floor isolation of a building is made according to the invention, the thermal insulation material is advantageously complemented with activated carbon, whose function is to adsorb the radon gas emanating from the ground and retain it until the radioactivity of the radon gas has decayed to an insignificant level. Advantageously, the activated carbon is dispersed as homogeneously as possible among the base material fibers to maximize the statistical possibilities of adsorbing radon atoms.

The activated carbon is advantageously admixed with the fibers by approx. 1 - 20 %, advantageously 1 - 5 %, of the base material fiber weight, while the anhydrous inorganic agent capable of later accumulating water of hydration is used by 2 - 8 % of the base material fiber weight, and both of these agents are admixed with the fibrous base material prior to the milling step. Subsequent to the milling step, the hydrous portions of the fire-retardant agents can be admixed with the material in a conventional manner.

Owing to its nonsettling structure, the thermal insulation material according to the invention can also be used for insulating vertical walls by, e.g., blowing the organic fiber-based insulation material into the wall cavity.

### Example

Organic fiber-based products suited for use as thermal insulation were manufactured from recycled paper chiefly comprising newsprint. The recycled paper was first ripped into coarse shreds, after which to the paper-based material was added anhydrous borax by 2 - 8 % of the fibrous base material weight. The admixed material was defibered in a disk refiner equipped with grooved bars into a relatively coarse fluff having a particle size of approx. 1 - 5 mm. Subsequently the fluff was admixed with hydrous borax by 12 - 20 % of the fibrous base material weight.

For comparison, a reference fluff was prepared in which all the borax was admixed in hydrous form after the milling step.

Tests performed on the materials indicated that fire-retardant agents introduced in dry, anhydrous, fine-pulverized form later absorbed water of hydration, and resultingly, the settling of these insulation materials in vertical cavities was as little as only approx. 5 - 20 % of the settling of the comparative insulation material in which all of the fire-retardant agent was admixed in hydrous form after the milling step of the fibrous base material.

## Claims

1. A method of manufacturing an essentially fire-retardant product from a fibrous base material, according to which method
- the base material is defibered to a desired degree of defibering and
- a fire-retardant agent is admixed with it,
**characterized** by
- milling the fibrous base material in a refiner equipped with grooved bars in order to defiber the fibers,
- using as fire-retardant agents inorganic salts which absorb water of hydration in them and occur in both hydrous and anhydrous forms, and
- introducing 1/4 to 1/2 of the fire-retardant agent in anhydrous form prior to defibering and introducing 1/2 to 3/4 of the fire-retardant material to the fibrous base material after defibering in hydrous form.

2. A method as defined in claim 1, **characterized** by using at borax, soda or a combination thereof as fire-retarding material.

3. A method as defined in claim 1, **characterized** by performing the milling with a disk or conical refiner.

4. A method as defined in claim 1, **characterized** by complementing or augumenting the fire-retardant agents by other salts occurring in anhydrous and hydrous forms to the end of bonding other substances to the fibers.

5. A method as defined in claim 1, **characterized** by admixing the anhydrous fire-retardant agent with the fibrous base material by not more than approx. 10 to 15 %, advantageously not more than 8 %, of the base material fiber dry weight.

6. A method as defined in claim 1, **characterized** by complementing the defibering of the anhydrous agent to the base material with the milling of activated carbon to the fibers by approx. 1 to 20 % of the base material fiber weight.

7. Use of the method defined in claim 1 in the production of thermal insulation materials or aggregates for asphalt and similar coatings to be applied in hot form.

8. A thermal insulation material, **characterized** in that it has been prepared acccording to claim 1.

9. A thermal insulation material as defined in claim 8, **characterized** in that the fire-retardant agents are comprised of salts capable of absorbing at least five waters of hydration as well as occurring in anhydrous form or forms of a smaller amount of water of hydration.

10. A thermal insulation material as defined in claim 8, **characterized** in that the salts used as fire-retardant agents are capable of releasing an essential fraction of their water of hydration at a temperature higher than 30 °C yet lower than 120 °C.

11. A thermal insulation material as defined in claim 8, **characterized** in that it contains 1 to 20 % pulverized activated carbon based on the dry weight of the fibers.

12. A thermal insulation material as defined in claim 8, **characterized** in that it contains besides salts acting as fire-retardant agents also other anhydrous and hydrous salts capable of bonding other materials to the fibers.

13. A thermal insulation material as defined in claim 8, **characterized** in that it comprises recycled paper shredded to a fluff with a particle size of approx. 0.1 to 50 mm, advantageously 1 to 10 mm, admixed with borax, soda or a mixture thereof.

14. A thermal insulation material as defined in claim 13, **characterized** in that the fibers are defibered from at least essentially wood-fiber-containing recycled paper.

15. An aggregate for asphalt and similar coatings applied in hot form, **characterized** in that is has been prepared according to claim 1.

16. An aggregate as defined in claim 15, **characterized** in that the fibers are essentially comprised of defibered organic fibers milled to a particle size of approx. 0.01 to 10 mm, advantageously 0.1 to 5 mm, said organic fibers being defibered from recycled paper containing mineral fillers.

17. An aggregate as defined in claim 16, **characterized** in that it incorporates as mineral fillers approx. 1 to 50 % clay and/or talc.

## Patentansprüche

1. Verfahren zur Herstellung eines im wesentlichen feuerbeständigen Produktes aus einem Material auf Faserbasis, wobei nach diesem Verfahren
- das Basismaterial bis zu einem bestimmten Entfaserungsgrad entfasert wird und
- ein feuerhemmendes Mittel zugemischt wird,
dadurch gekennzeichnet, daß
- das Material auf Faserbasis in einem Refiner, der mit geriffelten Stäben zum Entfasern der Fasern ausgerüstet ist, gemahlen wird,
- als feuerhemmendes Mittel ein anorganisches Salz verwendet wird, das Hydratwasser aufnimmt und sowohl in Hydrat als auch in Anhydridform auftritt, und
- 1/4 bis 1/2 des feuerhemmenden Mittels in Anhydridform vor der Entfaserung zugegeben wird, und
- 1/2 bis 3/4 des feuerhemmenden Materials in Hydratform nach dem Entfasern zu dem Material auf Faserbasis zugegeben wird.

2. Verfahren nach Anspruch 1, dadurch gekennzeichnet, daß als feuerhemmendes Material Borax, Soda oder eine Kombination daraus verwendet wird.

3. Verfahren nach Anspruch 1, dadurch gekennzeichnet, daß das Mahlen mit einem Scheiben- oder Konus-Refiner durchgeführt wird.

4. Verfahren nach Anspruch 1, dadurch gekennzeichnet, daß die feuerhemmenden Mittel durch andere Salze, die als Hydrat in Anhydridform auftreten, nach dem Einbinden anderer Substanzen in die Fasern ergänzt oder verbessert werden.

5. Verfahren nach Anspruch 1, dadurch gekennzeichnet, daß das wasserfreie feuerhemmende Mittel mit dem Material auf Faserbasis zu nicht mehr als 10 bis 15 %, vorteilhafter Weise nicht mehr als 8 % des Fasenrockengewichts des Basismaterials vermischt wird.

6. Verfahren nach Anspruch 1, dadurch gekennzeichnet, daß das Entfasern des wasserfreien Mittels zu dem Basismaterial mit dem Vermahlen von Aktivkohle zu den Fasern in etwa 1 bis 20 Gew.-% des Basisfasermaterialgewichtes ergänzt wird.

7. Verwendung des Verfahrens nach Anspruch 1 für die Herstellung von thermischem Isolationsmaterial oder Aggregate für Asphalt und ähnliche Beschichtungen, die in heißer Form aufgebracht werden.

8. Thermisches Isolationsmaterial, dadurch gekennzeichnet, daß es nach Anspruch 1 hergestellt wurde.

9. Thermisches Isolationsmaterial nach Anspruch 8, dadurch gekennzeichnet, daß die feuerhemmenden Mittel aus Salzen bestehen, die sowohl dazu fähig sind, zumindest 5 Hydratwassermoleküle zu absorbieren, als auch in Anhydridform aufzutreten, oder in einer Form mit geringeren Mengen von Hydratwasser.

10. Thermisches Isolationsmaterial nach Anspruch 8, dadurch gekennzeichnet, daß die als feuerhemmenden Mittel verwendeten Salze dazu fähig sind, eine wesentliche Menge ihres Hydratwassers bei einer Temperatur oberhalb von 30°C, aber niedriger als 120°C freizulassen.

11. Thermisches Isolationsmaterial nach Anspruch 8, dadurch gekennzeichnet, daß es 1 bis 20% pulverisierte Aktivkohle, bezogen auf das Trockengewicht der Fasern, enthält.

12. Thermisches Isolationsmaterial nach Anspruch 8, dadurch gekennzeichnet, daß es neben den als feuerhemmende Mittel wirkenden Salzen auch andere wasserfreie oder wasserhaltige Salze enthält, die dazu fähig sind, andere Materialien an die Fasern zu binden.

13. Thermisches Isolationsmaterial nach Anspruch 8, dadurch gekennzeichnet, daß es Recyclingpapier enthält, das zu einem Flaum mit einer Teilchengröße von etwa 0,1 bis 50 mm, vorteilhafterweise 1 bis 10 mm zerkleinert und mit Borax, Soda oder einer Mischung daraus vermischt wurde.

14. Thermisches Isolationsmaterial nach Anspruch 13, dadurch gekennzeichnet, daß die Fasern von zumindest im wesentlichen Holzfasern enthaltendem Recyclingpapier entfasert werden.

15. Aggregat für Asphalt und ähnliche Beschichtungen, die in heißer Form angewendet werden, dadurch gekennzeichnet, daß es nach Anspruch 1 hergestellt wurde.

16. Aggregat nach Anspruch 15, dadurch gekennzeichnet, daß die Fasern im wesentlichen aus entfaserten organischen Fasern bestehen, die zu einer Teilchengröße von etwa 0,01 bis 10 mm, vorteilhafterweise 0,1 bis 5 mm zermahlen wurden, wobei die genannten organischen Fasern aus Recydingpapier, das Mineralfüllstoffe enthält, entfasert wurden.

17. Aggregat nach Anspruch 16, dadurch gekennzeichnet, daß es als Mineralfüller etwa 1 bis 50 % Tonerde und/oder Talg enthält.

## Revendications

1. Procédé de fabrication d'un produit pratiquement non inflammable, à partir d'un matériau de base fibreux, procédé selon lequel
- le matériau de base est défibré jusqu'à un certain degré de défibrage, et
- et un agent non inflammable lui est incorporé,
caractérisé par :
- le broyage du matériau de base fibreux dans un raffineur équipé de barreaux cannelés afin de défibrer les fibres,
- la mise en oeuvre, en tant qu'agents non inflammables, de sels minéraux qui absorbent l'humidité, et se présentent à la fois sous forme anhydre et sous forme hydratée, et
- l'introduction, avant le défibrage, du quart à la moitié, de la quantité de l'agent non inflammable sous forme anhydre, et
- l'incorporation au matériau de base après le défibrage, de la moitié aux trois-quarts, de la quantité de l'agent non inflammable sous forme anhydre.

2. Procédé selon la revendication 1, caractérisé par l'emploi du borax, de la soude, ou d'une combinaison des deux, en tant qu'agent non inflammable.

3. Procédé selon la revendication 1, caractérisé par la mise en oeuvre du broyage à l'aide d'un raffineur à disque ou conique.

4. Procédé selon la revendication 1, caractérisé par l'action de compléter ou d'augmenter les agents non inflammables, par d'autres sels se présentant sous forme anhydre ou hydratée, dans le but de lier d'autres substances aux fibres.

5. Procédé selon la revendication 1, caractérisé par le mélange de l'agent non inflammable anhydre, au matériau de base fibreux, à raison d'environ 10 à 15 %, avantageusement à raison de pas plus de 8 %, par rapport au poids de fibres de matériau de base, exprimé en sec.

6. Procédé selon la revendication 1, caractérisé par l'action de compléter la défibration de l'agent non inflammable ajouté au matériau de base, par le broyage de charbon activé ajouté aux fibres à raison d'environ 1 à 20 %, par rapport au poids de fibre de matériau de base.

7. Utilisation du procédé selon la revendication 1, pour la production de matériaux d'isolation thermique, ou d'agrégats pour asphalte et revêtements similaires, destinés à être appliqués à chaud.

8. Matériau d'isolation thermique caractérisé en ce qu'il a été préparé selon la revendication 1.

9. Matériau d'isolation thermique selon la revendication 8, caractérisé en ce que les agents non inflammables sont composés de sels capables d'absorber au moins cinq eaux d'hydratation, ainsi que de se présenter sous forme anhydre, ou hydratée avec une faible quantité d'eau d'hydratation.

10. Matériau d'isolation thermique selon la revendication 8, caractérisé en ce que les sels utilisés comme agents non inflammables, sont capables de libérer une fraction essentielle de leur eau d'hydratation à une température supérieure à 30°C, mais cependant inférieure à 120°C.

11. Matériau d'isolation thermique selon la revendication 8, caractérisé en ce qu'il contient 1 à 20 % de charbon actif pulvérisé, par rapport au poids sec des fibres.

12. Matériau d'isolation thermique selon la revendication 8, caractérisé en ce qu'il contient aussi, en plus des sels agissant comme agents non inflammables, d'autres sels anhydres et hydratés, capables de fixer d'autres matériaux aux fibres.

13. Matériau d'isolation thermique selon la revendication 8, caractérisé en ce qu'il contient du papier recyclé déchiqueté sous la forme d'un duvet de taille de particules comprise entre environ 0,1 à 50 mm, avantageusement entre 1 et 10 mm, mélangé à du borax, à de la soude, ou à un mélange des deux.

14. Matériau d'isolation thermique selon la revendication 13, caractérisé en ce que les fibres sont défibrées à partir d'un papier recyclé contenant essentiellement de la fibre de bois.

15. Agrégat pour asphalte et revêtements similaires appliqués à chaud, caractérisés en ce qu'ils ont été préparés selon la revendication 1.

16. Agrégat selon la revendication 15, caractérisé en ce que les fibres se composent essentiellement de fibres organiques défibrées, broyées à une taille de particules comprise approximativement entre 0,010 et 10 mm, avantageusement entre 0,1 et 5 mm, lesdites fibres organiques étant défibrées à partir de papier recyclé contenant des charges minérales.

17. Agrégat selon la revendication 16, caractérisé en ce qu'il comprend, en tant que charges minérales, 1 à 50 % d'argile et/ou de talc.
